

## UNITED STATES PATENT OFFICE

2,649,415

## CORROSION INHIBITOR COMPOSITION

Robert L. Sundberg, Phillipsburg, N. J., Charles P. Albus, Easton, Pa., and James M. Cross, Belvidere, N. J., assignors to General Aniline & Film Corporation, New York, N. Y., a corporation of Delaware

No Drawing. Application December 30, 1949,  
Serial No. 136,172

13 Claims. (Cl. 252—8.55)

1

This invention relates to corrosion inhibiting compositions for use in acid baths employed in metal treatment, particularly for iron and steel. The invention also relates to the acid baths employed for such treatment, containing the corrosion inhibitors of the invention, and to metal treatment processes employing the same.

Metal pickling involves treatment of a metal such as iron or steel with a strong acid bath to remove surface impurities such as oxide scale formed thereon in the course of manufacture. Since the strong acids employed are capable of attacking the metal itself, it is advantageous to add to the bath a corrosion inhibitor which enhances the selective action of the acid on the surface impurities, and substantially reduces or prevents attack of the metal by the acid.

Another field of metal treatment employing strong aqueous acids is in "acidizing" treatment of oil wells. A strong aqueous mineral acid is introduced into the oil well to increase the flow of oil by attacking the underground porous rock formations containing the oil. Since the acid solutions come in contact with metal equipment of the well, it is advantageous to incorporate a corrosion inhibitor in the acid solution to prevent excessive damage of the metal equipment. Another problem arising in acidizing treatment of oil wells lies in the resolution or inhibition of oil-in-water emulsions which normally tend to form during and as a result of the acidizing treatment. For this purpose, numerous surface-active agents have been suggested for incorporation in the well treating fluid. For example, it has been suggested in USP 2,233,383 to employ water-soluble non-ionic surface-active polyglycol ethers, prepared by reaction of ethylene oxide on a water-insoluble acyclic alcohol, as an emulsion breaker in the acidizing of oil wells. As indicated in this patent, prevention of corrosion of the metal equipment by the acids employed calls for the additional use of a corrosion inhibitor.

Higher primary aliphatic and alicyclic amines, especially monoamines, which are at most slightly soluble in water, and particularly those containing 12 to 20 carbon atoms, have some corrosion inhibiting action in acid solutions, but are generally only partially effective to prevent substantial corrosion when employed in the low concentrations (of the order of 0.01 to 0.20%) in which they can be incorporated in acid solutions with satisfactory economy and without substantial separation of solids.

We have discovered that mixtures of higher primary aliphatic or alicyclic amines with water-

2

soluble non-ionic emulsifying agents of the type containing a polyalkylene glycol ether radical of at least 4 oxyalkylene radicals, attached by an ether or carboxy ester linkage to a higher aliphatic, alicyclic or alkylated aromatic hydrocarbon radical of at least 12 (e. g. 12 to 24 carbon atoms), and wherein the weight ratio of said amine to said emulsifying agent is substantially within the range 1:9 to 1:1, and preferably about 1:3, are highly effective corrosion inhibitors for ferrous metals such as iron and steel, unexpectedly exceeding the inhibiting effect of their respective components when used in strong acid solutions (e. g. solutions of a pH less than 2) in concentrations of the order of 0.01 to 0.20%.

The corrosion inhibitor compositions of this invention are soluble or readily dispersible in strong aqueous acid solutions, and can be readily compounded to avoid undesirable separation of solids from the solution during use in metal treatment.

The corrosion inhibiting mixtures of this invention are highly effective in the acid baths employed for pickling which contain, for example, sulfuric, hydrochloric, nitric, hydrofluoric, phosphoric, formic or acetic acid in concentrations of about 5 to 15%, or in equivalent aqueous solutions of acid salts such as sodium bisulfate. They are also effective and useful as corrosion inhibitors in the acidizing of oil wells with strong acids (e. g. hydrochloric or hydrofluoric acid) of 5 to 20% concentration, wherein the corrosion inhibiting compositions also act to prevent or inhibit formation, and to resolve, water-in-oil emulsions.

As indicated above, the amines employed in the compositions of this invention are aliphatic and alicyclic primary monoamines of 12 to 20 carbon atoms, particularly the primary amines derived from fatty acids of natural fats by replacement of the carboxyl group with an amino or an amino methyl group, and the alicyclic primary monoamines derived from rosin or its hydrogenated or dehydrogenated derivatives, e. g. by replacing carboxyl groups with an amino methyl group in abietic or hydrogenated or dehydrogenated abietic acid, or by introducing a primary amino group into the nucleus of abietyl compounds and their hydrogenated or dehydrogenated derivatives, e. g. by nitration and reduction as disclosed in USP 2,367,001, or by halogenation and amination as disclosed in USP 2,240,936.

The non-ionic emulsifying agents employed in the corrosion inhibitor compositions of this in-

vention are water-soluble or colloidally soluble polyglycol ethers and esters of higher fatty or alicyclic alcohols or carboxy acids, and of alkylphenols, of the order of 12 to 24 carbon atoms, which are produced by condensation of such acids, phenols or alcohols with at least 4 molecular equivalents of ethylene oxide or a closely analogous alkylene oxide such as propylene oxide. Preparation of such compounds is disclosed, for example in USP 1,970,578.

The following compositions, prepared in each case by thoroughly mixing the ingredients here given, and warming until a homogeneous mixture was obtained, illustrate a number of representative corrosion inhibiting compositions in accordance with our invention. Parts are by weight.

- (a) 50 parts of polyethoxylated talloil
- 50 parts of dehydroabietinyl amine
- (b) 75 parts of polyethoxylated talloil
- 25 parts of dehydroabietinyl amine
- (c) 75 parts of polyethoxylated di-isoamylphenol
- 25 parts of dehydroabietinyl amine
- (d) 75 parts of polyethoxylated talloil
- 25 parts of a straight-chain aliphatic primary amine mixture of 14 to 18 carbon atoms
- (e) 90 parts of polyethoxylated talloil
- 10 parts of dehydroabietinyl amine

Talcol is a byproduct of the sulfate process for making wood pulp, the crude product usually consisting of rosin acids (30 to 65%) and fatty acids (40 to 60%), and the refined product containing, for example 35 to 40% of rosin acids and 50 to 60% of higher fatty acids, together with up to about 10% unsaponifiable ingredients.

The polyethoxylated derivatives employed in the foregoing compositions contain 4 or more, and particularly from 8 to 15 ethoxy radicals, and are prepared by condensing ethylene oxide in the appropriate molecular proportions with talloil or with the di-isoamylphenol. Similar compositions are obtained by using a similar ethylene oxide derivative of nonyl phenol, or a condensation product of about 50 mols of ethylene oxide with one mol of talloil.

Dehydroabietinyl amine is a primary amine derivative of dehydroabietic acid in which the carboxyl group is replaced by  $-\text{CH}_2-\text{NH}_2$  group. In the following table, it is called "rosin amine." The straight-chain aliphatic amine of the foregoing compositions, derived from natural fat fatty acids of 14 to 18 carbon atoms, is prepared, for example, by amination of the fatty alcohol mixture obtained by reduction of esters of fatty acids, or by catalytic hydrogenation of the corresponding nitriles.

The corrosion inhibiting effect of the foregoing compositions, and also of the respective components of said compositions, was tested by incorporating the inhibiting compositions and the respective ingredients alone, in concentrations of 0.01, 0.10 and 0.20%, in 15% aqueous hydrochloric acid at 80° C., and determining the loss in weight during 15 minutes immersion in the resulting solutions, of approximately equal-sized samples of  $\frac{1}{8}$ -inch hot rolled steel sheets, and comparing the per cent loss in weight with the corresponding loss of a similar sample in hydrochloric acid of the same temperature and concentration and in the absence of any inhibitor. The loss in weight of the latter blank determination amounted to 3.874%.

Inhibiting efficiency was calculated in percent-

age as the quotient of the difference in loss in weight between the sample with the inhibitor and without the inhibitor, over the loss in weight in the absence of an inhibitor.

The results of the tests were as follows:

| 10  | Inhibitor Composition |         |            |             | Inhibitor Efficiency—Concentration in 15% HCl |       |       |
|-----|-----------------------|---------|------------|-------------|-----------------------------------------------|-------|-------|
|     | Amines                |         | Polyethoxy |             | 0.01%                                         | 0.10% | 0.20% |
|     | Rosin                 | Fatty   | Talloil    | Alk. Phenol |                                               |       |       |
| 15  | Percent               | Percent | Percent    | Percent     | 89                                            | 98    | 98    |
| (a) | 50                    | 50      | 75         | —           | 82                                            | 98    | 98    |
| (b) | 25                    | —       | —          | 75          | 82                                            | 98    | 98    |
| (c) | 25                    | —       | —          | 90          | 84                                            | 96    | 96    |
| (d) | —                     | 25      | 75         | —           | 67                                            | 96    | 97    |
| (e) | 10                    | —       | —          | 100         | 9                                             | 77    | 98    |
| 20  | 100                   | —       | —          | 100         | 11                                            | 30    | 71    |
| 25  | —                     | —       | —          | —           | 51                                            | 73    | 74    |
| 30  | —                     | —       | —          | 100         | 25                                            | 58    | 63    |

Similar inhibitor efficiencies were obtained with corresponding mixtures of polyethoxylated nonyl phenol or ethoxylated talloil containing about 50 molecular equivalents of ethylene oxide with the rosin amine or the fatty amine mixture.

As indicated in the foregoing table, the corrosion inhibiting effect of mixtures of the higher fatty and alicyclic amines with polyalkylene glycol esters and ethers substantially exceeds the corrosion inhibiting effect of either of the ingredients when used in corresponding concentrations alone. In the instance of rosin amine, which attained 98% efficiency at 0.2% concentration when used alone, the insolubility of the material at this concentration, and the resulting separation of solids, would render its use impractical for commercial application. However, mixtures containing 50% or more of the polyglycol ethers or esters with the insoluble amines yield stable dispersions or solutions in the strong acid medium employed, and are satisfactory for use in metal pickling baths or in acidizing oil wells.

As set out above, the amines employed in accordance with this invention are substantially water-insoluble (i. e., water-insoluble or at most, slightly water-soluble) higher primary aliphatic and alicyclic monoamines, especially those containing about 12 to 20 carbon atoms, such as primary amines derived from the fatty acids of natural fats, from the carboxy acids of rosin, e. g. abietic acid and its hydrogenated and dehydrogenated derivatives, and the like. The polyalkoxylated compounds employed in the corrosion inhibiting compositions are those derived from the fatty acids of natural fats or from the corresponding alcohols, from abietic acid and its hydrogenated or dehydrogenated derivatives or rosin, or from alcohols corresponding to the latter compounds, and from alkylphenols of at least 12 and preferably 12 to 24 carbon atoms. The number of mols of ethylene or propylene oxide condensed with these materials to produce the polyalkoxylated compounds should be at least 4 in order to afford satisfactory surface-active properties. The upper limit of the molecular proportion of alkylene oxide thus condensed is such that the products remain colloidally soluble in water. In general, up to 60 mols of ethylene oxide has been found suitable.

The proportions of the amine to the polyglycol ether compounds in corrosion inhibiting mixtures should be substantially within the range of 1:1 to 1:9. Substantially higher proportions of amine cause undesirable separation of solids in acid

baths, while with lower proportions of amine, the corrosion inhibiting effect decreases excessively.

The compositions are suitably employed in strong acid baths used for metal pickling or oil well treatment most advantageously and economically in concentrations of 0.01 to 0.2%. The baths may contain 5 to 20% of a mineral acid such as HCl, H<sub>2</sub>SO<sub>4</sub>, H<sub>2</sub>F<sub>2</sub>, H<sub>3</sub>PO<sub>4</sub>, HNO<sub>3</sub>, or in some cases, organic acids such as formic or acetic acid. Such baths have a pH of less than 2 and generally less than 1. In pickling operations, elevated temperatures of the order of 80° C., e. g. 50 to 100° C., are employed, and the bath is preferably maintained in motion relative to the metal articles to be treated. In the acidizing of oil wells, mineral acids, especially hydrochloric or hydrofluoric acid are used in concentrations of 5 to 20%, and the solution is not heated, but is introduced at ambient temperature into the oil well. When employed in the oil well treating solutions, the corrosion inhibiting compositions of the invention not only inhibit corrosion of the metal equipment, but also inhibit formation of water-in-oil emulsions.

Variations and modifications which will be obvious to those skilled in the art can be made in the foregoing compositions and procedure without departing from the nature or scope of the invention.

We claim:

1. A corrosion inhibiting composition for use in the treatment of metals with acid baths, which consists essentially of a substantially water-insoluble primary amine of the class consisting of aliphatic and alicyclic monoamines of 12 to 20 carbon atoms, and a non-ionic dispersing agent of the class consisting of the polyalkoxylated derivatives of aliphatic and alicyclic monocarboxy acids, of aliphatic and alicyclic monohydric alcohols and of alkylphenols, said acids, alcohols and alkylphenols having 12 to 24 carbon atoms, said derivatives thereof containing at least 4 oxyalkylene radicals and said oxyalkylene radicals each containing 2 to 3 carbon atoms, the weight ratio of said amine to said dispersing agent being substantially within the range of 1:1 to 1:9.

2. A corrosion inhibiting composition as defined in claim 1, wherein the dispersing agent is 50 polyethoxylated talloil.

3. A corrosion inhibiting composition as defined in claim 1, wherein the dispersing agent is a polyethoxylated alkylphenol.

4. A corrosion inhibiting composition as defined in claim 1, wherein the amine is a dehydroabietinyl amine. 55

5. A corrosion inhibiting composition as de-

fined in claim 1, wherein the amine is a higher fatty amine corresponding to a natural fat fatty acid.

5 6. A corrosion inhibiting composition essentially consisting of dehydroabietinyl amine and polyethoxylated talloil, wherein the weight ratio of said amine to said talloil derivative is about 1:3.

10 7. A corrosion inhibiting composition consisting of polyethoxylated di-isoamylphenol and dehydroabietinyl amine, wherein the weight ratio of said amine to said phenol derivative is about 1:3.

15 8. A corrosion inhibiting composition consisting essentially of a mixture of straight-chain aliphatic primary monoamines of 14 to 18 carbon atoms and of a polyethoxylated talloil, wherein the weight ratio of said amine mixture to said talloil derivative is about 1:3.

20 9. An acid treatment bath for metals, having a pH of less than 2 and containing from 0.01 to 0.2% of a corrosion inhibiting composition as defined in claim 1.

25 10. An acid treatment bath for metals, containing 5 to 20% of a mineral acid and from 0.01 to 0.2% of a corrosion inhibiting composition as defined in claim 1.

30 11. An acid treatment bath for metals, containing about 15% hydrochloric acid and from 0.01 to 0.2% of a corrosion inhibiting composition as defined in claim 1.

35 12. A process for pickling iron and steel, which comprises immersing the metal in an acid bath having a pH less than 2 and containing from 0.01 to 0.2% of a corrosion inhibiting composition as defined in claim 1.

40 13. A process for the treatment of oil wells having ferrous metal equipment therein, which comprises introducing into the well an acid bath containing 5 to 20% of a mineral acid and from 0.01 to 0.2% of a corrosion inhibiting composition as defined in claim 1, wherein said ferrous metal equipment is exposed to contact with said bath. 45

ROBERT L. SUNDBERG.  
CHARLES P. ALBUS.  
JAMES M. CROSS.

References Cited in the file of this patent

UNITED STATES PATENTS

| Number    | Name                  | Date          |
|-----------|-----------------------|---------------|
| 1,970,578 | Schoeller et al. ---- | Aug. 21, 1934 |
| 2,233,383 | De Groote et al. ---- | Feb. 25, 1941 |
| 2,246,842 | De Groote et al. ---  | June 24, 1941 |
| 2,367,001 | Campbell -----        | Jan. 9, 1945  |
| 2,510,063 | Bried -----           | June 6, 1950  |